

## UNITED STATES PATENT OFFICE

2,518,109

## PICKLING OF METALS

Richard O. Zerbe, Nitro, W. Va., assignor to Monsanto Chemical Company, St. Louis, Mo., a corporation of Delaware

No Drawing. Application July 2, 1947,  
Serial No. 758,729

18 Claims. (Cl. 252—150)

1

The present invention relates to the cleaning of metallic surfaces and particularly to a new class of steel pickling inhibitors which are employed to prevent undue attack upon the surface of a metal when in contact with a pickling bath of an acid nature.

Pickling solutions for removing oxides from the surface of metals ordinarily consist largely of a dilute solution of an inorganic acid such as sulfuric or hydrochloric acid. The acid although it dissolves the oxides and scale, also attacks the metal to some extent so that the acid is largely consumed and a certain amount of metal is lost. It also appears that the hydrogen liberated by the action of the acid on the metal has a serious embrittling effect upon the metal being treated. The escaping hydrogen also carries with it a fine spray of the acid liquor from the pickling bath which produces an atmosphere possessing corrosive properties and one which is injurious to health and damaging to equipment.

By the present invention, these objectionable features of the pickling process are substantially overcome or reduced to a minimum. More specifically, some of the objects of the present invention are to obviate over-pickling, embrittlement and pitting of the articles treated; to minimize the amount of metal lost in pickling; to increase the efficiency of the pickling operation; to prolong the effective life of the pickling bath; and particularly to facilitate the pickling operation. Other and further objects of the invention will be apparent from the following description and accompanying examples.

To accomplish to as great an extent as possible the objects set forth in accordance with the present invention, there is added to the pickling bath an inhibitor or regulating agent which acts to restrain the action of the acid from attacking clean metal but assists in removing the rust, scale, and other deposits or in other words the inhibitor causes the acid selectively to remove such materials without appreciably attacking the clean portions of the metal under treatment.

The new class of pickle regulators comprise 2-alkyl-mercaptoarylenethiazoles in which the alkyl group bears a terminal hydroxyl group and preferably contains one or more ether linkages. A general formula for the class of products of this invention is



2

where Ar is an ortho arylene radical, R is an alkylene group and n is an integer.

The new inhibitors may be prepared by introducing into mercaptoarylenethiazoles one or 5 more hydroxy alkyl radicals. Examples of suitable arylene thiazoles from which the new inhibitors may be prepared are 2-mercaptopbenzothiazole, 2-mercaptopnaphthothiazole, 2-mercaptop-4-phenylbenzothiazole, 2-mercaptopchlorobenzothiazole, and 2-mercaptoptolylthiazole.

Condensation of mercaptoarylenethiazoles may be effected with ethylene oxide, propylene oxide, glycide, epichlorhydrin, glycol, glycerine, polyglycerine, and the like. Two or more of these 15 reactive compounds may also be caused to react consecutively. The condensation is advantageously carried out in the presence of alkaline reacting agents or nickel sulfate as catalysts.

An important attribute of the new inhibitors is 20 their ready solubility in the pickling baths. The problem of dispersing insoluble inhibitors is a troublesome one and the presence of undissolved particles in the cleaning bath frequently results in spotting and staining of the metal pieces. 25 While all of the new inhibitors are at least partially soluble in acid pickling baths, those containing approximately four ether linkages are completely soluble. They produce a clear haze-free pickling bath. In addition, the presence of 30 at least one ether group in the molecule increases the inhibiting strength. Therefore, compounds where n in the foregoing general formula is greater than unity are preferred. Solubility determinations carried out in cold dilute acid with 35 condensation products of mercaptobenzothiazole and ethylene oxide revealed that the solubility in acid gradually increased with increasing values of n. Products in which the value of n was approximately 10 or more were completely soluble in cold 2% hydrochloric or sulfuric acid. In general, products in which the value of n is at least 5 but less than 31 are completely soluble in hot pickling baths in the amounts normally used.

40 It is usually preferred to employ between about one hundredth of one percent and three hundredths of one percent by weight based on the pickling bath. However, the composition, concentration, temperature of operation, and other 45 factors vary with different baths and similarly the optimum concentration of inhibitor will vary somewhat depending upon the particular conditions employed. The concentration of inhibitor based on the quantity of 100 per cent acid contained in the pickling bath is usually between 50

about two tenths of one percent and half of one percent.

2-hydroxy ethyl mercaptoarylenethiazoles may be prepared by reacting a 2-mercaptoproarylenethiazole with ethylene oxide in an inert organic solvent as described in co-pending application Serial No. 674,928 of Paul M. Downey, filed June 6, 1946. This application has matured into Patent No. 2,513,922. The following is a typical method of preparation.

Substantially 344 parts by weight of mercapto-benzothiazole was dissolved in 350 parts by weight of dioxane. A small amount of Nuchar or other absorptive carbon was added and ethylene oxide passed into the solution at 96-105° C. When ethylene oxide no longer continued to be absorbed, the black and small amounts of other insoluble material were filtered from the hot solution. The solvent was removed either by vacuum stripping or washing and drying and the residue heated up to 90° C. under 5 mm. vacuum. The product consisted of a light colored heavy viscous oil which set to a waxy solid on standing. After recrystallization from benzene the product melted at 52.5-54.5° C.

Other solvents may be used if desired, as for example monochlorobenzene, ortho dichlorobenzene, tetrachlorobenzene, and diethyl Carbitol.

Products soluble in dilute mineral acids under conditions of the pickling operation may be formed by condensing ethylene oxide either in gaseous or liquid form with molten 2-mercaptoprobenzothiazole and continuing the reaction until more than 5 but less than 30 mols of ethylene oxide have combined with each mol of mercapto-benzothiazole. These products and their preparation are disclosed and claimed in application Serial No. 758,719, filed of even date herewith in the name of Earl W. Gliesenkamp and assigned to the same assignee as the present case. This application has matured into Patent No. 2,498,617.

As exemplary of inhibitors containing at least one ether group, a series of products was prepared by reacting mercapto-benzothiazole with ethylene oxide in varying ratios. 172 parts by weight of 97% mercapto-benzothiazole (substantially one molecular proportion) and 0.9 part by weight of powdered KOH were charged into a suitable reaction vessel fitted with an alkylene oxide inlet tube and ethylene oxide run into the

In this manner a series of compounds was prepared possessing the structural formula

5



where  $n$  represents an integer. While  $n$  is a whole number in the case of any given molecule, it is convenient to designate  $n$  as a function of the average molecular weight and more particularly the total molecular weight equivalents of ethylene oxide actually reacted with each molecular weight of mercapto-benzothiazole. Accordingly, the value of " $n$ " in the table below is the number of moles of ethylene oxide reacted per mole of mercapto-benzothiazole and therefore assumes fractional values.

As specific embodiments of the invention which are to be understood as illustrative of the invention and not limitative thereof, typical examples of the preferred class of materials were employed in the metal pickling process under conditions which duplicated, so far as possible those commonly followed in commercial practice. A portion of one of the preferred class of compounds was incorporated in a pickling bath and its value as an inhibitor determined in the following manner: A test piece of 28 gauge hot rolled tin plate steel stock, approximately 4" x 3" in dimension, was immersed in the pickling bath comprising substantially 750 cc. of a water solution containing approximately 6% by weight of 66° Bé. sulfuric acid and a small amount of one of the inhibitors above described. The temperature of the bath was maintained at substantially 80° C. The steel test piece after thoroughly cleaning and pre-pickling for a few minutes in the absence of inhibitor and drying was weighed before immersion in the bath, and after 40 minutes pickling the test piece was again weighed, the difference between the two weights representing the metal loss during pickling. The metal loss compared with the metal loss of a similar test piece treated in an analogous manner but without the use of any inhibitor provides a measure of the inhibiting value of the compound employed. The results obtained on testing typical examples of the preferred class of materials are given in the following table. The metal loss is reported as the average of duplicate determinations.

Table

| Value of $n$         | Total Amount Grams | Solubility in pickling Bath at 80° C. | Loss of metal in Grams | Condition of Test Strips After Pickling |
|----------------------|--------------------|---------------------------------------|------------------------|-----------------------------------------|
| Blank - no inhibitor | .0986              | melted and gradually dissolved        | .7897                  | pitted.                                 |
| 1                    | .234               | do                                    | .0555                  |                                         |
| 1                    | .0936              | oily droplets                         | .0351                  |                                         |
| 3.6                  | .0936              | slight haze                           | .0096                  | spotted.                                |
| 3.6                  | .234               | do                                    | .0079                  | Do.                                     |
| 4.86                 | .0936              | do                                    | .0076                  | clean.                                  |
| 4.86                 | .234               | do                                    | .0072                  | very slight streaking.                  |
| 7.70                 | .0936              | completely soluble                    | .0117                  | clean.                                  |
| 7.70                 | .234               | do                                    | .0102                  | Do.                                     |
| 9.65                 | .0936              | do                                    | .0097                  | Do.                                     |
| 9.65                 | .234               | do                                    | .0094                  | Do.                                     |
| 15                   | .0936              | do                                    | .0103                  | Do.                                     |
| 15                   | .234               | do                                    | .0086                  | Do.                                     |

molten mixture at 204° C. Samples were taken at intervals and tested for their inhibiting value.

It is apparent from the data set forth that the preferred class of materials constitute an im-

portant and highly efficacious group of inhibitors as in all cases wherein one of the preferred inhibiting compounds was incorporated in the pickle liquor there resulted a great saving in the loss in weight of the steel test strips as compared with that resulting when no inhibitor was employed.

Other modes of employing inhibitors of the class hereinbefore set forth in the acid pickling of metals are apparent to those skilled in the art to which the invention pertains. The products described may be employed in the presence of foaming agents, ionizable substances or other materials ordinarily used. Thus the preferred class of materials may be employed as the sole inhibitor or they may be employed in conjunction with other materials exhibiting an inhibiting action or with inert fillers, dispersing agents, etc. Other non-oxidizing mineral acids than sulfuric acid may be employed in the pickle bath. Thus hydrochloric acid as well as other inorganic acids may be employed in the pickle bath in conjunction with the preferred class of inhibitors in the manner hereinbefore set forth.

What is claimed is:

1. A process of pickling a ferrous metal which comprises subjecting the metal to be pickled to the action of a heated nonoxidizing mineral acid solution containing about 0.2 to 0.5 percent by weight based upon 100 percent acid of a compound of the structure



where Ar is an ortho arylene radical, R is an alkylene radical and n is an integer greater than one but less than thirty-one.

2. A process of pickling a ferrous metal which comprises subjecting the metal to be pickled to the action of a heated nonoxidizing mineral acid solution containing about 0.2 to 0.5 percent by weight based upon 100 percent acid of a compound of the structure



where Ar is an ortho arylene radical, R is an alkylene radical of less than four carbon atoms and n is an integer greater than one but less than thirty-one.

3. A process of pickling a ferrous metal which comprises subjecting the metal to be pickled to the action of a heated nonoxidizing mineral acid solution containing about 0.2 to 0.5 percent by weight based upon 100 percent acid of a compound of the structure



where Ar represents an ortho arylene radical and n is an integer greater than one but less than thirty-one.

4. A process of pickling a ferrous metal which comprises subjecting the metal to be pickled to the action of a heated nonoxidizing mineral acid solution containing about 0.2 to 0.5 percent by weight based upon 100 percent acid of a compound of the structure



where n is an integer greater than one but less than thirty-one.

5. A process of pickling a ferrous metal which comprises subjecting the metal to be pickled to the action of a heated nonoxidizing mineral acid solution containing about 0.2 to 0.5 percent by weight based upon 100 percent acid of a compound of the structure



where n is an integer greater than five but less than thirty-one.

6. A process of pickling a ferrous metal which comprises subjecting the metal to be pickled to the action of a heated non-oxidizing mineral acid solution containing about 0.2 to 0.5 percent by weight based upon 100 percent acid of a compound of the structure



where n is an integer not less than ten but less than thirty-one.

7. A process of pickling iron and steel products which comprises subjecting the metal to be pickled to the action of a heated sulfuric acid solution containing about 0.2 to 0.5 percent by weight based upon 100 percent acid of a compound of the structure



where n is an integer greater than five but less than thirty-one.

8. A process of pickling iron and steel products which comprises subjecting the metal to be pickled to the action of a heated sulfuric acid solution containing about 0.2 to 0.5 percent by weight based upon 100 percent acid of a compound of the structure



where n is approximately ten.

9. A mineral acid pickling bath for metal products which comprises a nonoxidizing mineral acid solution containing a small proportion sufficient to inhibit the action of the acid on ferrous metals of a compound of the structure



where Ar is an ortho arylene radical, R is an alkylene radical and n is an integer greater than one but less than thirty-one.

10. A mineral acid pickling bath for metal products which comprises a nonoxidizing mineral acid solution containing a small proportion sufficient to inhibit the action of the acid on ferrous metals of a compound of the structure



where Ar is an ortho-arylene radical; R is an alkylene radical of less than four carbon atoms and n is an integer greater than one but less than thirty-one.

11. A mineral acid pickling bath for metal products which comprises a nonoxidizing mineral acid solution containing a small proportion sufficient to inhibit the action of the acid on ferrous metals of a compound of the structure



where Ar represents an ortho-arylene radical and n is an integer greater than one but less than thirty-one.

12. A mineral acid pickling bath for metal products which comprises a nonoxidizing mineral acid solution containing a small proportion sufficient to inhibit the action of the acid on ferrous metals of a compound of the structure



where n is an integer greater than one but less than thirty-one.

13. A mineral acid pickling bath for metal products which comprises a nonoxidizing mineral acid solution containing a small proportion sufficient to inhibit the action of the acid on ferrous metals of a compound of the structure



where n is an integer greater than five but less than thirty-one.

14. A mineral acid pickling bath for metal products which comprises a non-oxidizing mineral acid solution containing a small proportion sufficient to inhibit the action of the acid on ferrous metals of a compound of the structure



where n is an integer not less than ten but less than thirty-one.

15. A mineral acid pickling bath for metal products which comprises a sulfuric acid solution containing a small proportion sufficient to

inhibit the action of the acid on ferrous metals of a compound of the structure



where n is an integer greater than five but less than thirty-one.

16. A mineral acid pickling bath for metal products which comprises a sulfuric acid solution containing a small proportion sufficient to inhibit the action of the acid on ferrous metals of a compound of the structure



where n is approximately ten.

17. A process of pickling iron and steel products which comprises subjecting the metal to be pickled to the action of a heated hydrochloric acid solution containing about 0.2 to 0.5 percent by weight based upon 100 percent acid of a compound of the structure



where n is an integer greater than five but less than thirty-one.

18. A mineral acid pickling bath for metal products which comprises a hydrochloric acid solution containing a small proportion, sufficient to inhibit the action of the acid on ferrous metals, of a compound of the structure



where n is an integer greater than five but less than thirty-one.

RICHARD O. ZERBE.

#### REFERENCES CITED

The following references are of record in the file of this patent:

#### UNITED STATES PATENTS

| Number    | Name           | Date          |
|-----------|----------------|---------------|
| 1,990,963 | Teppema        | Feb. 12, 1935 |
| 2,383,681 | Pinkney et al. | Aug. 28, 1945 |